

Patented June 2, 1931

1,807,621

# UNITED STATES PATENT OFFICE

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MASSACHUSETTS

## SHOE STIFFENER AND PROCESS OF MANUFACTURE

No Drawing.

Application filed September 12, 1923. Serial No. 662,224.

This invention relates to shoe stiffening material such as is formed from fibrous sheet material saturated with thermo-plastic substances, that is, substances which at atmospheric and body temperature are rigid but which become soft and pliable when moderately heated, such as various compounds and mixtures of asphaltic and bituminous material, gums, resins, or kindred substances.

10 Particularly where such material is to be used for the manufacture of box toes it should be capable when softened of being stretched evenly and shaped to the toe without danger of tearing. For this reason the cheaper 15 grades of felt such as produced on a paper machine are not suitable, a felted material such as is produced by felting machines being much more satisfactory, though adding materially to the cost of the stiffener.

20 Machines for effecting the fabrication of felt such as heretofore used for box toes are bulky and slow in operation, the fibers from which the felt is made being shaken together and gradually reduced from a relatively thick 25 sheet to the much more densified sheet material in the finished felt. The process is long and slow and requires careful handling throughout by skilled workmen.

30 The object of this invention is to provide a stiffening material of which the fibrous base may be made on a paper machine and composed of such material as shall be eminently suited, because of its strength, porosity, and ability to withstand the forming operations about the last, without tearing or being otherwise injured. By producing the material on a paper machine it may be manufactured with great rapidity and with a comparatively simple mechanism and with but little expense for labor due to the relatively great output of a single paper machine. This is made possible by forming the material with a large proportion of goat or cattle hair which is preferably so treated as to be retained in its original length in the felt, without the formation of lumps or thick and thin spots in the felt.

45 A considerable quantity of hair of original length may be successfully incorporated in the felt provided a material is added which

is capable of individualizing the hair so that it may be separated and uniformly mixed in the pulp without the necessity of the hard beating ordinarily required. Such individualizing may be accomplished by the use of 55 slimy material such as short hair treated and beaten up hard with caustic soda until the hair is partially dissolved and reduced to a slimy mass also containing relatively short hair. To this mixture may be added the 60 long hair which may be individualized thereby and distributed throughout the mass. The beater roll may be so adjusted as to comb out the long hair without cutting it, so that practically all of it may finally appear in the 65 felted product in its original length. The method and furnishes for accomplishing this are more fully described and claimed in my application for patent Serial Number 662,220 filed September 12, 1923, for hair felt and 70 method of making. For example, rags, sulphate or sulphite pulp, and rags and wood flour, or combinations thereof, 20 parts by weight, and 30 parts of goat or cattle hair and 6 to 10 parts of caustic soda together with 75 water are beaten out hard for 20 minutes in the beater, the hair being beaten out short and reduced to a slimy mass. The beater roll is then raised slightly and 50 parts of long hair are added and the beating continued sufficiently hard to comb out the hair without cutting it until it is thoroughly individualized. 10 parts of alum are then added to 80 precipitate the dissolved hair.

In place of the mixture of short hair and 85 caustic soda, leather dissolved in caustic soda may be employed. The leather may be dissolved in the caustic and the solution added to the beater or the leather may be placed in the beater in the form of chips or skivings 90 and the caustic allowed to act thereon during the beating operation. This also forms a slimy mass which is capable of individualizing the long hair which is later added thereto. This method and the furnish are more 95 fully described and claimed in my application for Patent Serial Number 662,222 filed September 12, 1923, for hair felt and method of making.

Still another method of individualizing 100

the long hair consists in mixing a solution of soap or saponified oils or fatty acids with the long hair. This latter method produces a felt capable of having a greater proportion of hair of original length than the two previous methods. For example, 15 to 20 parts of cellulose fiber such as sulphate, rags, cotton, linters, etc., or combinations thereof, are beaten out for about 15 minutes. The beater roll is then raised and hair from 50 to 90 parts added, together with 20 parts of soap solution. This is circulated in the beater for about an hour with the beater roll sufficiently hard down to comb out the hair without cutting it until each fiber is coated with the individualizing agent. The pulp is then ready for the paper machine and should be run quite "wet" and under heavy suction. This method and furnish are more fully described and claimed in my application for patent Serial No. 662,221, filed September 12, 1923, for hair felt and method of making.

Where hair and caustic or a solution of leather are employed they may be precipitated in the final product by the alum or other precipitating agent and produce a harder and more dense product incapable of receiving as great a proportion of saturant as that produced by the use of the soap solution which is washed out in the felting operation. The soap might, also, however, be precipitated, if desired, by the use of alum, but this would not produce so hard a board as when short hair and caustic or leather solution is employed. Other materials which act to form a slimy mass in the beater engine such as talc or fine asbestos may also be used as the individualizing agent.

The hair felt is saturated with the thermoplastic material while in sheet form, the sheet being then cut to the required shape to form individual stiffener blanks which are skived to form the finished stiffeners.

The stiffener thus made is assembled with the upper of the shoe and then subjected to a temperature sufficiently high to soften the thermo-plastic saturant, whereupon the upper and the stiffener is shaped to the last, being pulled over and fastened to the sole or innersole of the shoe. During the pulling operation the stiffener stretches uniformly, the long hair fibers playing past each other while still retained firmly in felted condition by the saturant. The long hair prevents the material from tearing apart and as it is uniformly distributed the stretching and distortion takes place uniformly without the production of thick and thin spots, wrinkles, or creases. On subsequent cooling after the pulling over and lasting operations have been completed, the stiffener sets firmly to its molded form.

One very valuable characteristic of a stiffener made as hereinbefore described, particularly where soap is used as the individual-

izing agent for the long hair and is washed out with the wash water, the hair of original length representing from 70% to 90% of the felt, is that its surface is somewhat rough so that when the stiffener is heated the thermoplastic material flows between it and the adjacent shoe parts and acts as it hardens to firmly unite all the parts. There is thus no possibility of the shoe upper loosening from the stiffener when in use and wrinkling as sometimes happens when comparatively smooth surfaced material such as is formed from felt made on a felt machine is used. A stiffener made according to this invention is exceedingly well adapted for the use intended and is materially cheaper and more satisfactory than that having a felt base made on the usual felt machine.

I claim:

1. A shoe stiffener comprising a felt base including hair of original length, short hair, and insoluble gelatinous material fixed thereto, said base being saturated with thermoplastic material and cut and skived.

2. A process which comprises forming a stock containing cellulosic fiber, an individualizing agent, and a major portion of hair of original length, beating the stock to effect the combing and individualization of the hair but without substantially reducing its length, running the stock off on a paper machine to produce a porous felt, and filling the pores of the felt with a thermoplastic stiffening material.

3. A process of making shoe stiffeners, which comprises forming a stock containing cellulosic fiber, an individualizing agent, and a major portion of hair of original length, beating and combing out the hair until it is thoroughly individualized, precipitating the individualizing agent on the stock, running the stock off on a paper machine to produce a porous felt, saturating the felt with a thermoplastic stiffening material, and cutting the felt into shoe stiffener blanks.

4. A shoe stiffener felt including a cellulosic fiber, hair of original length, short hair, and dissolved hair precipitated thereon, said felt being saturated with thermoplastic material.

5. A process which comprises forming a stock containing cellulosic fiber, an individualizing agent and a major portion of hair of original length, beating the stock to effect the combing and individualizing of the hair but without substantially reducing its length, running the stock off on a paper machine to produce a porous felt, saturating the felt with a thermoplastic stiffening material, cutting the felt into shoe stiffener blanks, and skiving the blanks.

6. A process which comprises hard-beating hair in the presence of alkaline water until the hair is partially dissolved and reduced to a slimy mass containing relatively

short hair, adding hair of original length and cellulosic fiber, beating and combing out the long hair until it is thoroughly individualized, precipitating the dissolved hair on the stock, running the stock off on a paper machine to produce a porous felt, and saturating the felt with thermoplastic stiffening material.

5 In testimony whereof I have affixed my  
10 signature.

ALBERT L. CLAPP.

15

20

25

30

35

45

50

55

60

65